

July 18, 1961

J. L. MERO

2,993,122

METHOD OF ANALYZING URANIUM AND THORIUM ORES

Filed Dec. 23, 1957

10 Sheets-Sheet 1

FIGURE 1

THE GAMMA SPECTRUM OF AN EQUILIBRIUM URANIUM ORE



INVENTOR  
JOHN L. MERO

BY  
*Bruce & Brosler*  
ATTORNEYS

July 18, 1961

J. L. MERO

2,993,122

METHOD OF ANALYZING URANIUM AND THORIUM ORES

Filed Dec. 23, 1957

10 Sheets-Sheet 2

FIGURE 2

THE GAMMA-RAY SPECTRUM OF A URANIUM-RICH PLEISTOCENE GRAVEL URANIUM ORE DEPOSIT. THE GAMMA-RAY SPECTRA OF CHEMICALLY REFINED URANIUM SALTS ARE SIMILAR TO THIS GRAPH.



INVENTOR  
JOHN L. MERO

BY  
*Bruce & Brosler*  
ATTORNEYS

July 18, 1961

J. L. MERO

2,993,122

METHOD OF ANALYZING URANIUM AND THORIUM ORES

Filed Dec. 23, 1957

10 Sheets-Sheet 3

FIGURE 3

THE GAMMA-RAY SPECTRUM OF A RADIUM-RICH ORE. THIS SPECIFIC GRAPH IS OF A SULPHATE SCALE FOUND ON A WATER TROUGH NEAR A WATER WELL. THE NUCLIDES CAUSING THE PEAKS IN THIS GRAPH ARE PRINCIPALLY  $\text{Bi}^{214}$  AND  $\text{Pb}^{214}$ .



INVENTOR  
JOHN L. MERO

BY  
*Bruce & Broder*  
ATTORNEYS

July 18, 1961

J. L. MERO

2,993,122

METHOD OF ANALYZING URANIUM AND THORIUM ORES

Filed Dec. 23, 1957

10 Sheets-Sheet 4

FIGURE 4

THE GAMMA-RAY SPECTRUM OF A URANIUM-DEFICIENT ORE. SOME OF THE URANIUM GROUP OF NUCLIDES OF THE URANIUM DECAY SERIES ARE STILL ACTIVE AS EVIDENCED BY THE LARGE COUNT OF CHANNEL 1. TAILINGS FROM URANIUM CONCENTRATION PROCESSES HAVE A SIMILAR SPECTRUM.



INVENTOR  
JOHN L. MERO

BY  
*Bruce & Broder*  
ATTORNEYS

July 18, 1961

J. L. MERO

2,993,122

METHOD OF ANALYZING URANIUM AND THORIUM ORES

Filed Dec. 23, 1957

10 Sheets-Sheet 5

FIGURE 5a: THE GAMMA-RAY SPECTRUM OF THE RADIUM GROUP OF NUCLIDES.



FIGURE 5b: THE GAMMA-RAY SPECTRUM OF THE URANIUM GROUP OF NUCLIDES.



FIGURE 5c: THE GAMMA-RAY SPECTRUM OF THE COMBINED URANIUM AND RADIUM GROUPS FORMING AN EQUILIBRIUM ORE.



INVENTOR.  
JOHN L. MERO

BY  
*Bruce & Broder*

ATTORNEYS

July 18, 1961

J. L. MERO

2,993,122

METHOD OF ANALYZING URANIUM AND THORIUM ORES

Filed Dec. 23, 1957

10 Sheets-Sheet 6

FIGURE 6

THE GAMMA SPECTRUM OF AN EQUILIBRIUM URANIUM ORE WITH THE CHANNELS USED IN ANALYSIS INDICATED.



INVENTOR.  
JOHN L. MERO

BY  
*Bruce & Brodler*

ATTORNEYS

July 18, 1961

J. L. MERO

2,993,122

METHOD OF ANALYZING URANIUM AND THORIUM ORES

Filed Dec. 23, 1957

10 Sheets-Sheet 7

FIGURE 7

THE GAMMA-RAY SPECTRUM OF AN EQUILIBRIUM THORIUM ORE WITH THE CHANNELS USED IN ORE ANALYSIS INDICATED. THERE IS SOME URANIUM IN THIS ORE. THE ORE IS ABOUT 20 PARTS THORIUM TO 1 PART URANIUM.



INVENTOR.  
JOHN L. MERO

BY  
*Bruce & Broder*

ATTORNEYS

July 18, 1961

J. L. MERO

2,993,122

METHOD OF ANALYZING URANIUM AND THORIUM ORES

Filed Dec. 23, 1957

10 Sheets-Sheet 8

FIGURE 8

THE GAMMA-RAY SPECTRUM OF A CHEMICALLY REFINED THORIUM OXIDE THAT IS SEVERAL YEARS OLD. A COMPARISON OF THIS GRAPH WITH THE GRAPH OF AN EQUILIBRIUM THORIUM ORE SUCH AS THAT ILLUSTRATED IN FIGURE 7 INDICATES THAT THORIUM WILL ATTAIN A STATE OF NEAR EQUILIBRIUM VERY RAPIDLY.



INVENTOR  
JOHN L. MERO

BY  
*Bruce & Brosler*  
ATTORNEYS

July 18, 1961

J. L. MERO

2,993,122

METHOD OF ANALYZING URANIUM AND THORIUM ORES

Filed Dec. 23, 1957

10 Sheets-Sheet 9

FIGURE 9

THE GAMMA-RAY SPECTRUM OF A SAMPLE OF MATERIAL FROM A DEPOSIT OF THE RADIUM NUCLIDES AND THEIR DAUGHTERS OF BOTH THE URANIUM AND THE THORIUM DECAY SERIES. THE MOTHER NUCLIDES,  $U^{238}$  AND  $Th^{232}$ , ARE ABSENT FROM THIS MATERIAL.



INVENTOR  
JOHN L. MERO

By  
*Bruce & Brosler*  
ATTORNEYS

July 18, 1961

J. L. MERO

2,993,122

METHOD OF ANALYZING URANIUM AND THORIUM ORES

Filed Dec. 23, 1957

10 Sheets-Sheet 10

FIGURE 10

A PLOT OF THE CHANNEL 3-CHANNEL 4 COUNT RATE RATIO VERSUS THE RATIO OF THE PERCENT  $U_3O_8$  TO THE PERCENT  $ThO_2$  IN COMPOSITE ORES.



INVENTOR.  
JOHN L. MERO

BY  
*Bruce + Broder*

ATTORNEYS

## 1

2,993,122

METHOD OF ANALYZING URANIUM AND  
THORIUM ORES  
John L. Mero, 1823 Spruce St., Berkeley 9, Calif.  
Filed Dec. 23, 1957, Ser. No. 704,490  
4 Claims. (Cl. 250—83.3)

My invention relates to ore assaying and more particularly to a radiometric method of determining the equilibrium condition of naturally occurring radioactive ores, and determining ore grades.

Among the objects of my invention are:

- (1) To provide a novel and improved method of reliably assaying uranium and thorium ores;
- (2) To provide a novel and improved radiometric method for uranium and thorium ores;
- (3) To provide a novel and improved method for analyzing uranium and thorium ores, which method is relatively simple, reliable and applicable to automatic routine procedure;
- (4) To provide a novel and improved method which enables one to determine whether a specific uranium or thorium ore is in a state of radioactive equilibrium or not;
- (5) To provide a novel and improved method which enables one to determine the cause of non-equilibrium in a specific uranium and thorium ore;
- (6) To provide a novel and improved method which enables one to analyze uranium-thorium composite ores no matter what the equilibrium condition of the ore may be.

Additional objects of my invention will be brought out in the following description of a preferred embodiment of the same taken in conjunction with the accompanying drawings wherein,

FIGURE 1 is a graph depicting the gamma spectrum of an equilibrium uranium ore;

FIGURE 2 is a graph depicting the gamma-ray spectrum of a uranium-rich pleistocene gravel uranium ore deposit;

FIGURE 3 is a graph depicting the gamma-ray spectrum of a radium-rich ore;

FIGURE 4 is a graph depicting the gamma-ray spectrum of a uranium-deficient ore;

FIGURE 5a is a graph depicting the gamma-ray spectrum of the radium group of nuclides;

FIGURE 5b is a graph depicting the gamma-ray spectrum of the uranium group of nuclides;

FIGURE 5c is a view depicting the gamma-ray spectrum of the combined uranium and radium groups forming an equilibrium ore;

FIGURE 6 is a graph depicting the gamma-ray spectrum of an equilibrium uranium ore with the channels used in analysis indicated;

FIGURE 7 is a graph depicting the gamma-ray spectrum of an equilibrium thorium ore with the channels used in analysis indicated;

FIGURE 8 is a graph depicting the gamma-ray spectrum of a chemically refined thorium oxide that is several years old;

FIGURE 9 is a graph depicting the gamma-ray spectrum of a sample of material from a deposit of the radium nuclides and their daughters of both the uranium and the thorium decay series;

FIGURE 10 is a graph depicting the uranium-thorium ratio as a function of the ratio of gamma-ray energy emitted at key nuclides.

## 2

In its preferred form, my invention will be described principally as to its applicability to the assaying of radioactive ores such as uranium and thorium bearing ores.

## 5 RADIOACTIVE ORE ANALYSIS BY GAMMA-RAY SPECTROSCOPY

Radiometric methods of analyzing naturally occurring radioactive ores have not been accepted by industry as a means of analyzing ores on a routine basis because of a 10 lack of reliability of results. This lack of reliability in radiometric assays is due, largely, to a lack of radioactive equilibrium between the various nuclides in a decay series of a radioactive ore. If some method could be found to determine the equilibrium condition of an 15 ore, accurate and reliable assays could be obtained by radiometric methods.

The present invention provides a simple and sure 20 method for determining whether an ore is in a state of radioactive equilibrium or not; if not, the cause of the non-equilibrium can also be determined. Methods are then presented by which equilibrium ores and certain 25 non-equilibrium ores can be assayed.

The particular radiometric method of the present invention consists in measuring the intensity of the gamma 25 radiation of various energies emitted by specific nuclides in a radioactive ore. To do this a device called a gamma-ray scintillation spectrometer is used.

## 30 THEORY OF THE GAMMA-RAY SCINTILLATION SPECTROMETER

The gamma-ray scintillation spectrometer consists of 35 three principal units, a scintillation detector, a pulse height analyzer, and a scaler.

## The scintillation detector

When gamma radiation impinges on certain inorganic materials such as sodium iodide, the gamma photon is 40 absorbed by the crystal; in the place of the absorbed gamma ray a flash of light is emitted by the crystal. The intensity of this light is proportional to the energy of the absorbed gamma ray. Optically coupled to the NaI crystal is a photoelectric tube which converts the flash of light into an electric impulse. The voltage or height 45 of this impulse is proportional to the intensity of the light striking the cathode of the photoelectric tube and thus proportional to the energy of the absorbed gamma ray. After proper amplification this voltage impulse is fed into the pulse height analyzer.

## The pulse height analyzer

The pulse height analyzer is an electronic device that 50 contains a gating circuit which can be set to receive voltage pulses of a specific height. It accomplishes this by having two discriminators or thresholds. If the voltage 55 of the impulse is not high enough to reach the setting of the lower discriminator it is disregarded. If the voltage of the pulse exceeds the setting of the upper discriminator it is fed into an anticoincidence circuit which will cancel 60 the output of the discriminator. Only pulses which exceed the setting of the lower threshold but do not exceed the setting of the upper threshold are passed on to actuate a scaling mechanism. The voltage difference between the upper and the lower setting of the discriminator 65 is termed the window width of the analyzer. The particular voltage height that this window is set to intercept is termed a channel.

**3**  
*The scaler*

The scaler is another electronic device which simply counts the output pulses of the pulse height analyzer discriminator. The count collected by the scaler divided by the time over which the count was taken is a direct measure of the intensity of the gamma radiation of a particular energy being absorbed by the scintillation crystal.

The gamma radiation emitted by a particular nuclide or isotope is mono-energetic, thus, the gamma-ray spectrometer channel can be set to count the gamma rays coming from a particular nuclide. As the number of gamma rays per unit time is proportional to the amount of that nuclide present, a quantitative analysis can be made of the nuclide. In this way, by assaying an ore for key nuclides of the decay series, the state of the radioactive equilibrium of the ore can be determined.

**NATURAL RADIOACTIVITY**

All elements found in nature with atomic numbers greater than 83 (bismuth) are radioactive. A substance, or element, is radioactive when the atoms of which it is composed disintegrate spontaneously regardless of whether or not the emission of radiation can be readily detected in the process. In natural radioactive decay there are three types of rays that may be emitted, alpha rays, beta rays, and gamma rays.

Alpha rays are helium nuclei. They bear a positive charge equal in magnitude to that of two electrons. Beta rays, or beta particles, are negatively charged high speed electrons. Gamma rays are very short wave length electromagnetic radiations, the wave length of gamma radiation being several orders of magnitude shorter than that of visible light. Both alpha rays and beta rays are relatively easily absorbed in matter which makes the efficient detection of these particles for ore analysis under routine conditions often a difficult process. Gamma radiation, on the other hand, is not so easily absorbed; this makes detection of it under routine conditions a more convenient operation.

A radioatom in decaying may emit more than one gamma ray or it may emit none. In any case, no matter how many gamma rays are emitted, each gamma photon will have a characteristic wave length or energy. Table 1 and Table 2 list the nuclides of the two major natural radioactive decay series. Included in these tables are the gamma rays emitted by each nuclide.

TABLE 1.—THE URANIUM DECAY SERIES

| Name of Nuclide       | Atomic Number | Nuclide           | Half-Life                   | Energy of Gamma Rays Emitted by Nuclide (kev.) <sup>1</sup>                              |
|-----------------------|---------------|-------------------|-----------------------------|------------------------------------------------------------------------------------------|
| <b>Uranium Group:</b> |               |                   |                             |                                                                                          |
| Uranium I.....        | 92            | U <sup>238</sup>  | 4.5×10 <sup>9</sup> y.....  | 47 (?)                                                                                   |
| Uranium XI.....       | 90            | Th <sup>234</sup> | 24.1 d.....                 | 93                                                                                       |
| Uranium XZ.....       | 91            | Pa <sup>234</sup> | 1.18 m.....                 | 394, 782, 806, 820                                                                       |
| <b>Uranium II:</b>    |               |                   |                             |                                                                                          |
| Ionium.....           | 92            | U <sup>234</sup>  | 2.6×10 <sup>4</sup> y.....  | 60, 93, 118                                                                              |
| Ionium.....           | 90            | Th <sup>230</sup> | 8.0×10 <sup>4</sup> y.....  | 68, 140, 190, 228, 240                                                                   |
| <b>Radium Group:</b>  |               |                   |                             |                                                                                          |
| Radium.....           | 88            | Ra <sup>226</sup> | 1,600 y.....                | 188                                                                                      |
| Radon.....            | 86            | Rn <sup>222</sup> | 3.825 h.....                |                                                                                          |
| Radium A.....         | 84            | Po <sup>218</sup> | 3.05 m.....                 |                                                                                          |
| Radium B.....         | 82            | Pb <sup>214</sup> | 26.8 m.....                 | 53, 242, 259, 295, 351                                                                   |
| Radium C.....         | 83            | Bi <sup>214</sup> | 17.9 m.....                 | 68, 191, 426, 498, 609, 766, 933, 1,120, 1,238, 1,379, 1,520, 1,761, 1,820, 2,200, 2,420 |
| Radium C'.....        | 84            | Po <sup>214</sup> | 164×10 <sup>-6</sup> s..... |                                                                                          |
| Radium D.....         | 82            | Pb <sup>210</sup> | 22 y.....                   | 7, 23, 32, 37, 43, 47, 65                                                                |
| Radium E.....         | 83            | Bi <sup>210</sup> | 5.0 d.....                  |                                                                                          |
| Radium F.....         | 84            | Po <sup>210</sup> | 138 d.....                  | 84, 790                                                                                  |
| Radium G.....         | 82            | Pb <sup>206</sup> | Stable.....                 |                                                                                          |

<sup>1</sup> Branching decays of less than 0.1 percent are omitted.

**4**

TABLE 2.—THE THORIUM DECAY SERIES

|    | Name of Nuclide    | Atomic Number | Nuclide           | Half-Life                   | Energy of Gamma Rays Emitted by Nuclide (kev.) <sup>1</sup>                        |
|----|--------------------|---------------|-------------------|-----------------------------|------------------------------------------------------------------------------------|
| 5  | Thorium.....       | 90            | Th <sup>232</sup> | 1.4×10 <sup>10</sup> y..... | 55, 75                                                                             |
|    | Mesothorium 1..... | 88            | Ra <sup>228</sup> | 6.7 y.....                  | 30                                                                                 |
|    | Mesothorium 2..... | 89            | Ac <sup>228</sup> | 6.13 h.....                 | 60, 135, 184, 338, 462, 533, 590, 913, 969                                         |
| 10 | Radiothorium.....  | 90            | Th <sup>228</sup> | 1.9 y.....                  | 87                                                                                 |
|    | Thorium X.....     | 88            | Ra <sup>224</sup> | 3.64 d.....                 | 241                                                                                |
|    | Thoron.....        | 86            | Rn <sup>220</sup> | 54.5 s.....                 |                                                                                    |
|    | Thorium A.....     | 84            | Po <sup>216</sup> | 0.16 s.....                 |                                                                                    |
|    | Thorium B.....     | 82            | Pb <sup>212</sup> | 10.6 h.....                 | 115, 176, 238, 249, 299                                                            |
| 15 | Thorium C.....     | 83            | Bi <sup>212</sup> | 60.5 m.....                 | 40, 144, 164, 288, 328, 432, 452, 472, 720, 830, 1,030, 1,340, 1,610, 1,810, 2,200 |
|    | Thorium C'.....    | 84            | Po <sup>212</sup> | 0.3×10 <sup>-6</sup> s..... |                                                                                    |
|    | Thorium C'.....    | 81            | Tl <sup>208</sup> | 3.1 m.....                  | 277, 510, 582                                                                      |
| 20 | Thorium D.....     | 82            | Pb <sup>208</sup> | Stable.....                 | 859, 2,620                                                                         |

<sup>1</sup> Hollander, J. M., Perlman, I., and Seaborg, G. T., Tables of Isotopes: Rev. Modern Physics, v. 25, pp. 469-651, 1953.

*Radioactive decay*

The average time that a radioactive nucleus exists before it disintegrates into some other nucleus ranges greatly from one substance to another. The law that governs radioactive decay is exponential: consequently, it takes an infinitely long time for all of the atoms of any particular element to disintegrate. Because of this, a unit of time called the half-life is used to describe the rate of radioactive decay of a particular nuclide. The half-life is the length of time it will take for one-half of the initial atoms of a particular material to disintegrate. Thus only one-half of a sample of U<sup>238</sup> disappears by radioactive decay in  $4.5 \times 10^9$  years. In contrast to this, one-half of a sample of Po<sup>214</sup> disintegrates in  $10^{-4}$  seconds. Nothing can be done in any way to change the rate at which a given material will disintegrate. The half-life is independent of pressure, temperature, and other conditions under natural control.

*Radioactive equilibrium*

An atom that disintegrates to form another atom is called the parent and the product is called the daughter. A radio-atom is in a state of secular radioactive equilibrium with its disintegration product when the same number of atoms of the daughter nuclide disintegrate as are formed in a unit of time. Thus, in a radioactive decay series in equilibrium, the number of atoms of a nuclide being formed is exactly equal to the number of atoms of that nuclide disintegrating. Therefore, the number of disintegrations per unit time is the same for each member in the decay series. As all members of the decay series do not decay at the same rate, there will have to be a greater amount of the longer lived nuclides present to provide the same number of disintegrations per unit time as that coming from the shorter lived nuclides: consequently, the amount of a nuclide present in a decay series in equilibrium is directly proportional to its half-life.

A state of non-equilibrium exists when all or part of one or more of the daughters or parents is physically removed from the decay series. If a nuclide with a short half-life is removed, equilibrium can be rapidly regained. If a nuclide with a long half-life is removed, it may be millions of years before complete equilibrium is regained between all the members of the decay chain. After uranium is deposited it takes several millions of years to establish approximate equilibrium between all the members of the decay series mainly because of the long half-lives of two of the daughters of U<sup>238</sup>. A state of secular equilibrium, however, is regained between the first three members of the uranium group of the uranium decay series in less than a year. And assuming that U<sup>234</sup> has

the same chemical properties as  $U^{238}$  secular equilibrium is generally maintained between the first four members of the uranium series. At least in nature this should be true. As all of the daughters of  $Ra^{226}$  have short half-lives secular equilibrium is also maintained in this group of the uranium decay series when radium is present. When thorium is deposited it takes only a few decades to establish approximate radioactive equilibrium between all of the members of the decay series as all of the daughters of  $Th^{232}$  have relatively short half-lives.

#### EQUILIBRIUM AND NON-EQUILIBRIUM IN ORES

The various elements of a decay series have varying chemical properties. Uranium is generally more soluble in naturally occurring solutions than are the other elements of the uranium decay chain. If an ore deposit is exposed, and many of the Colorado Plateau ores are at or very near the surface, the natural processes of leaching can remove varying amounts of the valuable uranium content of the ore having a deposit deficient in this element. As most of the gamma radiation is emitted by the radium group of the uranium decay chain, such deposits can still be very radioactive.

A rather interesting process which will cause a state of non-equilibrium in ores is the migration of radon, a gas which is formed as the daughter of radium in the uranium decay series. It is not uncommon to find ore bodies that vary in the state of equilibrium from the bottom to the top of the deposit because of the upward migration of radon. Such a process would leave the bottom of the deposit deficient in the radium group of nuclides, the center of the deposit in an approximate state of equilibrium, and the top of the deposit with an excess of the radium group of nuclides.

Another type of radioactive deposit is that in which only the nuclides of the radium group of the uranium decay series are present. Many prospectors have discovered abnormal radioactivity at well heads or in hot springs deposits. Generally associated with this activity is a sulphate of barium or strontium. Radium, which has a half-life of 1600 years, is taken into solution with these sulphates and when these solutions come to the surface, the radium is precipitated along with the sulphates. Because of the short half-lives of the daughters of radium, secular equilibrium between the parent and daughter products is rapidly established. Inasmuch as some of the daughters of radium, notably  $Bi^{214}$  and  $Pb^{214}$ , are copious emitters of gamma radiation, the deposit will appear very radioactive. Seldom, however, do these ores contain uranium in commercial amounts.

In the uranium series the most important forms of non-equilibrium presently recognized are:

(1) Radium group deficiency due to migration of radon;

(2) Daughter-product deficiency due to a lack of time to reach equilibrium or due to differential leaching of the daughter-products; and

(3) Uranium deficiency due to differential leaching of uranium or deposition of daughter products only.

The key nuclides in a uranium ore, then, are  $U^{238}$  and  $Ra^{226}$ . The gamma radiation emitted by these nuclides, however, is so weak it cannot be readily resolved in a gamma spectrum of a uranium ore. A radiometric quantitative analysis is made, therefore, for nuclides which are copious emitters of gamma radiation and which in nature are in a state of secular equilibrium with these key nuclides; the abundance of the key nuclides is then inferred from this analysis.

#### Gamma-ray spectra

The gamma-ray spectrum of an equilibrium uranium ore is illustrated in FIGURE 1, while FIGURES 2, 3, and 4 illustrate the gamma-ray spectra of the most common types of non-equilibrium ores.

The method used to obtain the picture of the gamma-ray spectrum of an ore as illustrated in this application

is not the conventional method used in obtaining gamma-ray spectra curves with pulse height analyzers. Instead of sweeping the discriminator through the spectrum of voltage pulses by simultaneously lowering both voltage thresholds of the discriminator so as to maintain a constant window width and produce a linear array of the gamma energy versus the intensity of gamma radiation at a particular energy, the method used in the present invention was one of holding the discriminator at a fixed level and then amplifying the voltage pulses produced by the scintillation detector up through the discriminator by increasing the voltage on the photomultiplier dynodes. Because the amplification of voltages in the photomultiplier is an exponential function of the applied voltage to each dynode, an exponential array of the gamma-ray energy versus the intensity of gamma radiation at a particular energy is obtained. Such a method is very advantageous because it condenses the spectra in the high energy region where no important gamma-photon peaks occur while it spreads the spectra out in the low energy region where the gamma rays of interest in assaying occur. If at the same time the voltage pulses are being amplified up through the discriminator, the output pulses of the discriminator are fed into an ink recorder, a plot of the energy versus the intensity of the gamma-radiation at a particular energy can be made. This was the method employed in producing the gamma-ray spectra graphs depicted in the drawings.

#### URANIUM ORE ANALYSIS

FIGURES 5a, 5b, and 5c illustrate the gamma spectra of (1) the radium group of nuclides; (2) the uranium group of nuclides; and (3) the combined groups of an equilibrium ore. FIGURE 6 shows the spectrum of a uranium ore in equilibrium and indicates the gamma-ray energies or channels used in counting for ore analysis. Table 3 describes these peaks, the energy at which they occur, and the nuclides primarily responsible for producing them. FIGURE 7 shows the gamma-ray spectrum of a thorium ore with the same channels indicated.

TABLE 3.—CHANNELS USED IN COUNTING FOR ORE ANALYSIS

| Channel Number | Approximate Energy of Peak (kev.) | Nuclides Primarily Producing the Peak in the $U^{238}$ Series | Nuclides Primarily Producing the Peak in the $Th^{232}$ Series |
|----------------|-----------------------------------|---------------------------------------------------------------|----------------------------------------------------------------|
| 1              | 85                                | $Th^{234}$ , $U^{234}$ , $Pb^{214}$                           | $Th^{228}$ , $Th^{232}$ , $Ac^{228}$                           |
| 2              | 190                               | $Ra^{226}$ , $Th^{230}$                                       | $Ac^{228}$                                                     |
| 3              | 238                               | $Pb^{214}$                                                    | $Pb^{212}$                                                     |
| 4              | 351                               | $Pb^{214}$                                                    | $Bi^{212}$                                                     |
| 5              | 969                               | $Bi^{214}$                                                    | $Ac^{228}$                                                     |

The total count on any one of these channels does not come entirely from the nuclide primarily producing the peak. The resolution of the spectrometer is by no means sharp and as Table 1 and Table 2 indicate there are a multitude of other nuclides emitting gamma rays with energies near that which the channels listed in Table 3 are set to intercept. It may be assumed, however, that the majority of the gamma rays counted on a specific channel are from the nuclides indicated in Table 3. Back-scattered and Compton effect gamma rays may produce part of the low energy peaks, but as indicated in FIGURE 3 they have only a minor effect. Thus, with a uranium ore, the count rate, expressed in counts per second, on channel 3 is produced primarily by  $Pb^{214}$ . When thorium and uranium are present in the same ore the count on channel 3 is produced by  $Pb^{214}$  of the uranium decay series and by  $Pb^{212}$  of the thorium decay series. How much of the total count each nuclide produces can be determined by a method outlined later.

With uranium ores in a state of radioactive equilibrium, the count rate of any channel is proportional to the amount of  $U^{238}$  that is in the ore.

*The equilibrium factor*

If the graphs of the spectra of the various types of uranium ores are inspected it will be noticed that when uranium is present in the ore the count rate on channel 2 will exceed that of the count rate on channel 3. When the uranium is removed from an ore the count rate on channel 2 will be less than that of channel 3. The ratio of the count rate on channel 2 to that on channel 3 can thus be used to determine whether an ore contains any uranium ore or not. This ratio, the channel 2 count rate divided by the channel 3 count rate, is termed the "equilibrium factor." For uranium ores in a state of approximate radioactive equilibrium this ratio will be between the limits 1.10 and 1.30. If the uranium ore is not in a state of radio-active equilibrium the value of this ratio will be outside these limits. By the value of this ratio the cause of the non-equilibrium can also be determined. If the value of the equilibrium factor is greater than 1.30, the ore is uranium-rich. Generally, uranium-rich ores, those ores that consist primarily of the uranium group of nuclides of the uranium decay series, will have equilibrium factors with values greater than 3.0. Radium-rich ores, those ores that consist predominately of the radium group of the uranium decay series, will exhibit equilibrium factors less than 1.00, the value of the factor being between the limits 0.85 and 0.98 in most cases. Uranium-deficient ores, those ores that contain the radium group of nuclides and certain nuclides of the uranium group, namely  $\text{Th}^{234}$ ,  $\text{Pa}^{234}$ , and  $\text{Th}^{230}$ , will exhibit equilibrium factors with values in the range 0.90 and 1.00. Uranium-deficient ores are probably not very common in nature as  $\text{Th}^{234}$  and  $\text{Pa}^{234}$  have relatively short half-lives and will decay to an insignificant amount very rapidly without  $\text{U}^{238}$  to sustain them. This type of ore is best exemplified by the tailings from a uranium concentration process. Uranium-deficient ores can be distinguished from radium-rich ores as the count rate of channel 1 will exceed that of channel 2 for uranium-deficient ores, while the count rate of channel 1 will be less than that of channel 2 for radium-rich ores.

When thorium is present the value of the equilibrium factor will be between 1.10 and 0.30 depending on the amount of thorium that is present. For a pure thorium ore with no uranium decay series nuclides present the value of the equilibrium factor will be around 0.30. A method to determine how much thorium is present will be outlined later.

*Analysis of uranium ores*

When the numerical value of the equilibrium factor is in the range 1.10 to 1.30, indicating a state of radioactive equilibrium for uranium ores and the presence of none of the nuclides of the thorium decay series, the percent of uranium in the ore can be obtained by multiplying the count rate on channel 2,  $C_2$  after an adjustment has been made for the background count rate on this channel, by a factor to convert from the count rate to percent uranium. Assays of this type are usually expressed as percent  $\text{U}_3\text{O}_8$ ; the formula, therefore, is set up to yield this value. Mathematically:

$$\text{Percent of } \text{U}_3\text{O}_8 = x_u w_u g_u k_u C_2$$

where  $x_u$ ,  $w_u$ ,  $g_u$ , and  $k_u$  are sample self-absorption, sample weight, sample-tube geometry, and unit-conversion factors, respectively. For a particular set of counting conditions,  $w_u$ ,  $g_u$ , and  $k_u$  will be numerical constants. Therefore,  $w_u g_u k_u = K_{2U}$ , and

$$\text{Percent of } \text{U}_3\text{O}_8 = x_u K_{2U} C_2$$

The sample self-absorption of gamma-radiation factor,  $x_u$ , is a function of the amount of heavy elements in an ore and the absorption coefficient of these elements. In the case of uranium and thorium ores, therefore, it is a

function of the grade of the ore. As lead and uranium are the only heavy elements of any consequence in a uranium ore, the self-absorption factor can be evaluated by means of the following type of expression:

$$x_u = \frac{2}{e^{-\mu_1 t_1} + e^{-\mu_2 t_2}}$$

in which  $e$  is the base of the natural logarithms, 2.718,  $\mu_1$  is adsorption coefficient of lead and  $\mu_2$  is the absorption coefficient of uranium, and  $t_1$  and  $t_2$  are the thicknesses of lead and uranium in the sample, respectively. Because the lead and uranium atoms are diffused throughout the sample it would be very difficult to evaluate this term. In any case, the amount of lead and uranium in the sample would have to be known before hand, which, if it were, would eliminate the need for further analysis.

Fortunately, this correction is negligible for low grade ores, and in the higher grade ores it can be evaluated by means of a graph containing a plot of the count rate on a particular channel versus the correction factor for the count rate of that channel.

Because of their general low grade, this factor will not enter the problem with ores usually encountered in routine assaying in the United States. If the count rate of channel 2 is less than 125 counts per second, therefore, this factor,  $x_u$ , can also be considered a constant, the value of which is 1.00.

For ores of a grade below about 5 percent  $\text{U}_3\text{O}_8$ , then

$$\text{Percent of } \text{U}_3\text{O}_8 = K_{2U} C_2 \quad (1)$$

For the particular geometry and sample weight used in the methods described the value of  $K_{2U}$  was 0.0420.

The most prominent factors affecting the count rate obtained with a particular sample on channel 2 and channel 3 are ones of sample-scintillation tube geometry, sample self-absorption, and sample weight. The absorption of the gamma radiation in the aluminum shielding of the crystal will be slight as the shielding is very thin and the absorption coefficient of aluminum is small. In any case it will be a constant percentage of each gamma ray of a particular energy emitted by the sample. The same is true of the aluminum cup in which the sample is held. The air between the sample and the crystal will have even less effect than the aluminum in absorbing the gamma radiation from the sample.

If the geometry of the crystal-sample set-up is held constant, this factor will introduce no counting variations for which adjustments must be made. Also if the weight of the sample being analyzed is held at a constant value, no adjustments will have to be made for this factor. For assays listed in this report the sample size was 20.0 grams. The sample was placed in an aluminum cup 5.0 centimeters in diameter. The sample and cup were then centered on a cylindrical NaI crystal about 2 millimeters from the free face of the crystal. The crystal used in this research was a 1 inch by 1 inch NaI(Tl) Harshaw crystal optically mounted on 6292 Dumont photomultiplier tube. For the data used to illustrate the methods outlined, a window width of 0.5 volts was used.

If high grade ores are encountered, instead of making a self-absorption adjustment the sample can be diluted before assaying to a grade below 5 percent  $\text{U}_3\text{O}_8$ . In most cases silica is a good material with which to dilute the rich ores.

Table 4 contains a list of the results of a number of assays run on ores from western United States and Africa. Inasmuch as a majority of the ores that are assayed for tonnage calculations and for mill control are of the near equilibrium type of ore, this energy discrimination method will provide a fast, reliable, simple, and accurate assay for the uranium content of the ore. Equally important, the method provides a simple means of distinguishing non-equilibrium type ores when they are encountered.

## Non-equilibrium uranium ores

Of the non-equilibrium type uranium ores, the uranium-rich ores can be assayed by gamma-ray discrimination methods when the equilibrium factor is 3.0 or greater. The formula is the same as Formula 1, however, the proportionality factor in this case,  $K_{2U}$ , is 0.021 instead of 0.042. Again, as in the case of equilibrium ores, of a grade higher than 5 percent  $U_3O_8$  must be diluted or a sample self-absorption adjustment must be made.

Radium-rich and uranium-deficient ores are very difficult to analyze with any accuracy because of the intense radioactivity of this type of material in comparison with the uranium such an ore will contain; the uranium content being only a few hundredths of a percent in most cases.

Table 5 is a list of three equilibrium and sixteen non-equilibrium ores showing how the equilibrium factor is used to identify each type of ore.

TABLE 4.—ANALYSIS OF URANIUM EQUILIBRIUM ORE BY FORMULA 1

| Ore No. | C <sub>1</sub> | C <sub>2</sub> | C <sub>3</sub> | C <sub>4</sub> | Equilibrium Factor, C <sub>2</sub> /C <sub>3</sub> | Radio Assay, Percent U <sub>3</sub> O <sub>8</sub> | Chem. Assay, Percent U <sub>3</sub> O <sub>8</sub> | Remarks (Source of Ore)   |
|---------|----------------|----------------|----------------|----------------|----------------------------------------------------|----------------------------------------------------|----------------------------------------------------|---------------------------|
| A-1     |                | 9.76           | 8.37           |                | 1.17                                               | 0.410                                              | 0.407                                              | Big Indian Wash, Utah.    |
| A-2     |                | 14.39          | 11.77          |                | 1.22                                               | 0.603                                              | 0.601                                              | Do.                       |
| A-3     |                | 19.37          | 15.69          |                | 1.24                                               | 0.813                                              | 0.834                                              | Moab, Utah.               |
| A-4     |                | 3.90           | 3.52           |                | 1.11                                               | 0.164                                              | 0.170                                              | Standard Mines, Utah.     |
| A-5     |                | 6.17           | 5.47           |                | 1.13                                               | 0.259                                              | 0.251                                              | Blue Lizard Mine, Utah.   |
| A-6     |                | 5.22           | 4.55           |                | 1.15                                               | 0.219                                              | 0.224                                              | Hidden Splendor M., Utah. |
| A-7     |                | 2.40           | 2.13           |                | 1.13                                               | 0.101                                              | 0.100                                              | AEC Standard Ore.         |
| A-8     |                | 51.56          | 44.07          |                | 1.17                                               | 2.165                                              | 2.15                                               | Do.                       |
| A-9     |                | 8.67           | 7.45           |                | 1.16                                               | 0.364                                              | 0.374                                              | Big Indian Wash, Utah.    |
| A-10    |                | 10.68          | 9.00           |                | 1.19                                               | 0.448                                              | 0.452                                              | Hidden Splendor M., Utah. |
| A-11    |                | 6.05           | 5.09           |                | 1.19                                               | 0.254                                              | 0.25                                               | AEC Standard Ore.         |
| A-12    |                | 36.36          | 29.01          |                | 1.17                                               | 1.527                                              | 1.513                                              | Lisbon Uranium, Utah.     |
| A-13    |                | 100.65         | 88.55          |                | 1.14                                               | 4.23                                               | 4.29                                               | AEC Standard Ore.         |
| A-14    |                | 25.30          | 21.60          |                | 1.17                                               | 1.062                                              | 1.103                                              | Moab, Utah.               |

## ROUTINE CHEMICAL ASSAYS

|      |       |       |  |      |      |      |                  |
|------|-------|-------|--|------|------|------|------------------|
| A-15 | 19.19 | 16.55 |  | 1.16 | 0.69 | 0.59 | Cameron, Ariz.   |
| A-16 | 19.93 | 15.66 |  | 1.27 | 0.84 | 0.93 | Wolpinit, Wash.  |
| A-17 | 9.64  | 7.57  |  | 1.27 | 0.41 | 0.48 | Carlile, Wyo.    |
| A-18 | 22.29 | 17.97 |  | 1.24 | 0.95 | 0.94 | Uravan, Colo.    |
| A-19 | 3.62  | 2.90  |  | 1.25 | 0.15 | 0.18 | Carlile, Wyo.    |
| A-20 | 30.54 | 27.35 |  | 1.12 | 1.28 | 1.02 | Morocco, Africa. |

TABLE 5.—RECOGNITION OF EQUILIBRIUM AND NON-EQUILIBRIUM ORES BY EQUILIBRIUM FACTOR

| Ore No. | C <sub>1</sub> | C <sub>2</sub> | C <sub>3</sub> | C <sub>4</sub> | Equil. Factor, C <sub>2</sub> /C <sub>3</sub> | Comp. Ore Factor C <sub>3</sub> /C <sub>4</sub> | Radio Assay, Percent U <sub>3</sub> O <sub>8</sub> | Chem. Assay, Percent U <sub>3</sub> O <sub>8</sub> | Remarks (Type of Ore) |
|---------|----------------|----------------|----------------|----------------|-----------------------------------------------|-------------------------------------------------|----------------------------------------------------|----------------------------------------------------|-----------------------|
| B-1     | 27.46          | 39.56          | 41.98          | 70.71          | 0.96                                          | 0.59                                            | 0.00                                               | 0.002                                              | Radium-rich.          |
| B-2     | 26.18          | 35.33          | 36.73          | 62.74          | 0.94                                          | 0.59                                            | 0.18                                               | 0.15                                               | Do.                   |
| B-3     |                | 3.50           | 2.84           |                | 1.23                                          |                                                 | 0.22                                               | 0.15                                               | Equil. Ore.           |
| B-4     | 345.43         | 228.36         | 250.28         | 384.03         | 0.91                                          | 0.65                                            | 2.41                                               | 2.27                                               | Uran.-defic.          |
| B-5     |                | 11.48          | 2.41           |                | 4.76                                          |                                                 | 0.04                                               | 0.04                                               | Uran.-rich.           |
| B-6     | 100.00         | 47.80          | 140.60         | 55.51          | 0.34                                          | 2.53                                            | 13.5                                               | 14.0                                               | Thorium ore.          |
| B-7     |                | 62.52          | 9.87           |                | 6.34                                          |                                                 | 0.22                                               | 0.22                                               | Uran.-rich.           |
| B-8     | 16.06          | 8.71           | 9.50           | 15.20          | 0.92                                          | 0.63                                            | 1.17                                               | 1.17                                               | Uran.-defic.          |
| B-9     |                | 27.98          | 22.86          |                | 1.22                                          |                                                 | 1.00                                               | 1.00                                               | Equil. Ore.           |
| B-10    | 50.70          | 30.88          | 47.20          | 41.80          | 0.65                                          | 1.13                                            | 0.80                                               | 0.80                                               | U-Th Comp. Ore.       |
| B-11    | 44.50          | 27.21          | 28.98          | 36.40          | 0.94                                          | 0.80                                            | 1.00                                               | 1.00                                               | U-Th Comp. Ore.       |
| B-12    | 19.85          | 9.17           | 26.65          | 10.21          | 0.34                                          | 2.61                                            | 0.08                                               | 0.08                                               | U-Th Comp. Ore.       |
| B-13    | 97.52          | 122.66         | 180.94         | 195.03         | 0.65                                          | 0.93                                            | 0.01                                               | 0.01                                               | Th-U Ra-Groups.       |
| B-14    | 48.74          | 58.41          | 100.76         | 89.47          | 0.58                                          | 1.13                                            | 0.14                                               | 0.14                                               | Th-U Ra-Groups.       |
| B-15    | 17.21          | 9.86           | 10.26          | 16.35          | 0.96                                          | 0.63                                            | 1.40                                               | 1.40                                               | Mill Tails.           |
| B-16    |                | 6.58           | 0.86           |                | 7.66                                          |                                                 | 0.68                                               | 0.68                                               | Uran.-rich.           |
| B-17    |                | 14.53          | 11.82          |                | 1.28                                          |                                                 | 0.610                                              | 0.610                                              | Equil. Ore.           |
| B-18    | 155.68         | 203.15         | 312.32         | 308.20         | 0.65                                          | 1.01                                            | 0.00                                               | 0.00                                               | Th-U Ra-Groups.       |
| B-19    | 45.53          | 29.90          | 33.97          | 51.30          | 0.88                                          | 0.66                                            | 0.000                                              | 0.000                                              | Radium-rich.          |

## THORIUM ORE ANALYSIS

When the composite ore ratio of a radioactive ore has a value of 3.0 or greater, indicating a pure thorium ore with none of the uranium series of nuclides present, and the horium equilibrium factor, the channel 1 count rate produced by the thorium series nuclides, C<sub>1T</sub>, divided by the channel 3 count rate produced by the thorium

series nuclides, C<sub>3T</sub>, is greater than 0.40, the ore may be analyzed for its thorium content by multiplying the channel 3 count rate by a proportionality factor, K<sub>3T</sub>, to convert from count rate intensity to percent thorium. As the percent of thorium in an ore is generally expressed as percent ThO<sub>2</sub>, the formula will be set up to yield this value. Mathematically:

$$\text{Percent of ThO}_2 = x_t w_t g_t k_t C_3$$

where x<sub>t</sub>, w<sub>t</sub>, g<sub>t</sub>, and k<sub>t</sub> are sample self-absorption, sample weight, sample-tube geometry and unit-conversion factors, respectively. For a particular set of counting conditions and for ores of a grade below about 5 percent ThO<sub>2</sub> x<sub>t</sub>, w<sub>t</sub>, g<sub>t</sub>, and k<sub>t</sub> will be numerical constants, therefore: x<sub>t</sub>w<sub>t</sub>g<sub>t</sub>k<sub>t</sub> = K<sub>3T</sub>, and

$$\text{Percent of ThO}_2 = K_{3T} C_3 \quad (2)$$

For the particular geometry and sample weight used

in the methods described, the value of K<sub>3T</sub> was 0.0403. The same sample weight and tube-sample geometry conditions as were described in the analysis for uranium ores apply in the analysis for thorium ores. The reason for computing an extra thorium equilibrium factor is to check and see if it is only the nuclides after Th<sup>232</sup> that are present in the ore. The same processes that leach

the radium nuclides from a uranium ore can leach the radium nuclides from the thorium decay series and redeposit these nuclides elsewhere. As the first daughter of the thorium decay series, Ra<sup>228</sup>, has a half-life of 6.7 years, such a deposit can remain quite radioactive for a number of years without Th<sup>232</sup> to sustain it. Some of the count rate on channel 1 is produced by Th<sup>232</sup>; when it is not present in an ore the count rate on this channel is lessened. A computation of the thorium equilibrium factor will indicate this fact.

Because of the short-lives of all of the daughters of the thorium decay series, the mother isotope of the decay series, Th<sup>232</sup>, will probably never, in nature, occur free of any of its daughters in any appreciable amount as will uranium. This fact is illustrated by FIGURE 8 which shows the spectrum of a refined thorium oxide which is but a few years of age. Notice the close similarity between this spectrum and that of a thorium equilibrium ore as shown in FIGURE 7. This indicates that all the daughters of the thorium decay series reach a state of approximate secular equilibrium with their parents in a relatively short time.

As with uranium ores, the radium nuclides of the thorium series can be leached from the ore and redeposited elsewhere. This is indicated by FIGURE 9 which shows the spectrum of a material which contains the radium group of nuclides of both the thorium and uranium decay series. There is no measurable amount of Th<sup>232</sup> or U<sup>238</sup> present in this ore. It is this type of ore that the thorium equilibrium factor is used to guard against.

Sample-self absorption of the gamma radiation becomes noticeable in ores with a grade of ThO<sub>2</sub> greater than about 1 percent, but it is negligible until the grade of the ore reaches about 5 percent ThO<sub>2</sub>, except for channel 1. Gamma radiation on channel 1 is especially susceptible to absorption in the heavy elements in the ore because of its very low energy. In place of an adjustment of the count rates, the ore can be diluted with silica to a grade below 5 percent ThO<sub>2</sub>.

Also complicating thorium assays is the fact that thorium seldom occurs free of uranium in nature. This is indicated in Table 6 by the fact that the composite ore factor,  $C_3/C_2$ , seldom has a value of 3.0 or above. Because of this, Formula 3 was used to calculate the percent of ThO<sub>2</sub> of the ores listed in Table 6. Formula 3, however, reduces to Formula 2 when there is no uranium present in the ore.

The somewhat greater variance of the radiometric assay from the chemical assay in the case of thorium ores can be partially explained by the fact that accurate chemical assays for thorium are very difficult to obtain. It may be, of course, that the radiometric assay is at fault. In any case the results of Table 6 indicate that this method should be sufficiently accurate for routine laboratory assays.

TABLE 6.—THORIUM ORE ANALYSIS RESULTS

| Ore No.  | C <sub>1</sub> | C <sub>2</sub> | C <sub>3</sub> | C <sub>4</sub> | Equil. Factor, C <sub>2</sub> /C <sub>3</sub> | Comp. Ore Factor, C <sub>3</sub> /C <sub>4</sub> | Thorium Equil. Factor, C <sub>1</sub> /C <sub>3</sub> | Radio Assay, Percent ThO <sub>2</sub> | Chem. Assay, Percent ThO <sub>2</sub> | Chem. Assay, Percent U <sub>3</sub> O <sub>8</sub> |
|----------|----------------|----------------|----------------|----------------|-----------------------------------------------|--------------------------------------------------|-------------------------------------------------------|---------------------------------------|---------------------------------------|----------------------------------------------------|
| C-1----- | 15.38          | 6.09           | 17.90          | 7.73           | 0.34                                          | 2.32                                             | 0.74                                                  | 0.65                                  | 0.69                                  | Tr.                                                |
| C-2----- | 54.45          | 42.05          | 127.35         | 45.00          | 0.33                                          | 2.83                                             | 0.44                                                  | 4.88                                  | 5.00                                  |                                                    |
| C-3----- | 10.60          | 4.50           | 13.65          | 4.80           | 0.33                                          | 2.85                                             | 0.74                                                  | 0.52                                  | 0.40                                  | 0.01                                               |
| C-4----- | 25.40          | 12.51          | 34.40          | 13.72          | 0.36                                          | 2.51                                             | 0.64                                                  | 1.28                                  | 1.44                                  | 0.05                                               |
| C-5----- | 82.00          | 48.40          | 147.00         | 51.40          | 0.33                                          | 2.86                                             | 0.49                                                  | 5.65                                  | 5.36                                  | 0.02                                               |
| C-6----- | 17.44          | 8.07           | 24.95          | 8.12           | 0.32                                          | 3.07                                             | 0.65                                                  | 0.97                                  | 1.00                                  | 0.04                                               |
| C-7----- | 4.23           | 1.65           | 4.93           | 1.78           | 0.34                                          | 2.77                                             | 0.80                                                  | 0.19                                  | 0.20                                  | 0.01                                               |
| C-8----- | 9.43           | 4.00           | 12.65          | 4.15           | 0.32                                          | 3.05                                             | 0.69                                                  | 0.50                                  | 0.50                                  | 0.02                                               |
| C-9----- | 15.20          | 6.58           | 21.23          | 6.70           | 0.31                                          | 3.17                                             | 0.72                                                  | 0.85                                  | 0.80                                  | 0.03                                               |

## ANALYSIS OF URANIUM-THORIUM COMPOSITE ORES

Uranium-thorium composite ores also can be analyzed by gamma-ray discrimination methods. Because it may be difficult to determine beforehand the grade of the ore,

sample-self absorption corrections should be made when the count rates of channels 1 and 2 go above the values of 50 and 125 counts per second, respectively. The other alternative is to dilute the sample until these count rates falls below this value, the amount of silica added being carefully noted.

Composite uranium-thorium ores can be recognized by a uranium equilibrium factor,  $C_2/C_3$ , between the limits 1.10 and 0.30. As radium-rich and uranium-deficient ores also exhibit equilibrium factors in this range, an additional operation must be made to differentiate a composite ore from these two non-equilibrium uranium ores. This can be done by determining the count rate on channel 4 and calculating the channel 3-channel 4 count rate ratio. This ratio is called the composite ore factor. For a pure uranium ore the value of this ratio is approximately 0.62. This will apply whether the ore is uranium-deficient or radium-rich or an equilibrium uranium ore. As uranium-rich ores produce about the same count on channels 3 and 4, this type of material will have little effect on the value of the composite ore factor. For thorium ores the value of this ratio is approximately 3.0. Values of this ratio between the limits 0.6 and 3.0 indicate uranium-thorium composite ores.

In a composite ore the count rate on channel 3,  $C_3$ , after subtracting the background count, is due to the sum of the count rate of the uranium nuclides in the ore,  $C_{3U}$ , and the count rate of the thorium nuclides in the ore,  $C_{3T}$ . Or,  $C_3 = C_{3U} + C_{3T}$ . Assuming both the uranium and the thorium to be in a state of radioactive equilibrium:

$$C_3 = C_{3U} (\% U_3O_8) + C_{3T} (\% ThO_2)$$

Dividing by  $C_{3T}$  (% ThO<sub>2</sub>) yields:

$$\frac{C_3}{C_{3T} (\% ThO_2)} = \frac{C_{3U} (\% U_3O_8)}{C_{3T} (\% ThO_2)} + 1$$

and,

$$C_{3T} (\% ThO_2) = \frac{C_3}{\frac{C_{3U} (\% U_3O_8)}{C_{3T} (\% ThO_2)} + 1}$$

Therefore,

$$\text{Percent of ThO}_2 = \frac{C_3}{\frac{C_{3U} (\% U_3O_8)}{C_{3T} (\% ThO_2)} + K_{3T}} \quad (3)$$

If the thorium series is in a state of radioactive equilibrium, the radiometric percent of ThO<sub>2</sub> will be equal to the chemical percent of ThO<sub>2</sub>. Because of the short half-lives of all of the daughters of the thorium decay series, near secular equilibrium usually does exist in thorium ores. In any case whether the thorium in the composite ore is in a state of equilibrium with its daughters or not can be determined by calculating the thorium equilibrium factor. Although thorium, at least in nature,

will be in equilibrium with its daughters, the daughter products of the thorium decay series, as illustrated by FIGURE 9, can exist without being in equilibrium with their parent. The state of equilibrium of the uranium in the sample should have no effect on the thorium assay.

Equation 3 could not be solved if it were not for the fact that the uranium-thorium ratio,

$$\frac{\% \text{ U}_3\text{O}_8}{\% \text{ ThO}_2}$$

can be plotted as a function of the composite ore factor,  $C_3/C_4$ . This relationship is shown in FIGURE 10. By taking the ratio of the count rates of a composite ore on channel 3 and channel 4 and by use of FIGURE 10, the value of the uranium-thorium ratio can be determined and substituted in Equation 3. For a solution to Equation 3 such a substitution is made and the percent  $\text{ThO}_2$  in the ore can be calculated directly. Multiplying this value of the percent  $\text{ThO}_2$  in the sample by the uranium-thorium ratio will yield the equivalent percent  $\text{U}_3\text{O}_8$  in the sample. That is the amount of uranium that will be in the ore sample if the uranium group of nuclides is in equilibrium with the radium group of nuclides. As  $C_{3U}$  comes mainly from the nuclides of the radium group of the uranium decay series, the assay for thorium is not affected by any major state of non-equilibrium that might exist in the uranium part of the composite ore.

Before a uranium assay is determined, however, the equilibrium condition of the uranium in the ore should be checked. This can be done by calculating the count rate contribution of the thorium on channels 3 and 2 and subtracting this value from the total count rate of these channels. The remaining values are the count rate contributions of the uranium nuclides on these channels. These values can be used in a conventional way to determine the uranium equilibrium factor

$$\frac{C_{2U}}{C_{3U}}$$

If the value of this ratio is between the limits 1.10 and

TABLE 7.—RESULTS OF ASSAYS ON COMPOSITE ORES

| Ore No. | Channel Count Rates (c./s.) |        |        |        | Equilibrium Factor, $C_2/C_3$ | Composite Ore Factor, $C_3/C_4$ | Thorium Equil. Factor, $C_{1T}/C_{3T}$ | Uranium Equil. Factor, $C_{2U}/C_{3U}$ | Radio. Assay, Percent $\text{ThO}_2$ | Chem. Assay, Percent $\text{ThO}_2$ | (1) Radio. Assay, Percent $\text{U}_3\text{O}_8$ | (2) Radio. Assay, Percent $\text{U}_3\text{O}_8$ | Chem. Assay, Percent $\text{U}_3\text{O}_8$ |
|---------|-----------------------------|--------|--------|--------|-------------------------------|---------------------------------|----------------------------------------|----------------------------------------|--------------------------------------|-------------------------------------|--------------------------------------------------|--------------------------------------------------|---------------------------------------------|
|         | $C_1$                       | $C_2$  | $C_3$  | $C_4$  |                               |                                 |                                        |                                        |                                      |                                     |                                                  |                                                  |                                             |
| D-1     | 41.20                       | 24.87  | 24.28  | 34.25  | 1.02                          | 0.71                            | 0.93                                   | 1.11                                   | 0.11                                 | 0.10                                | 1.06                                             | 1.01                                             | 1.00                                        |
| D-2     | 44.50                       | 27.21  | 28.98  | 36.40  | 0.94                          | 0.80                            | 0.73                                   | 1.21                                   | 0.34                                 | 0.33                                | 1.00                                             | 1.04                                             | 1.00                                        |
| D-3     | 18.18                       | 13.02  | 37.55  | 13.42  | 0.35                          | 2.80                            | 0.41                                   | 1.43                                   | 1.44                                 | 1.13                                | 0.10                                             | 0.11                                             | 0.14                                        |
| D-4     | 104.78                      | 73.92  | 74.94  | 103.03 | 0.99                          | 0.73                            | —.49                                   | 1.15                                   | 0.57                                 | 0.43                                | 2.96                                             | 2.93                                             | 3.01                                        |
| D-5     | 64.05                       | 35.87  | 89.09  | 38.15  | 0.40                          | 2.34                            | 0.68                                   | 1.31                                   | 3.22                                 | 2.68                                | 0.43                                             | 0.51                                             | 0.46                                        |
| D-6     | 50.70                       | 30.88  | 47.20  | 41.80  | 0.65                          | 1.13                            | 0.50                                   | 1.30                                   | 1.02                                 | 1.00                                | 1.07                                             | 0.99                                             | 1.00                                        |
| D-7     | 45.60                       | 27.48  | 33.20  | 37.10  | 0.83                          | 0.90                            | 0.57                                   | 1.11                                   | 0.52                                 | 0.50                                | 0.99                                             | 1.00                                             | 1.00                                        |
| D-8     | 23.20                       | 12.22  | 28.88  | 12.89  | 0.42                          | 2.24                            | 0.66                                   | 1.48                                   | 1.03                                 | 1.00                                | 0.17                                             | 0.20                                             | 0.20                                        |
| D-9     | 97.52                       | 122.66 | 180.94 | 195.03 | 0.65                          | 0.93                            | —1.40                                  | 0.94                                   | Nil                                  | Nil                                 | 0.51                                             | 0.49                                             | 0.01                                        |
| D-10    | 25.32                       | 18.70  | 34.94  | 23.63  | 0.54                          | 1.50                            | 0.26                                   | 1.10                                   | 0.98                                 | 0.78                                | 0.51                                             | 0.49                                             | Nil                                         |
| D-11    | 48.74                       | 53.41  | 100.76 | 89.47  | 0.58                          | 1.13                            | —.73                                   | 0.75                                   | Nil                                  | Nil                                 | 1.84                                             | 1.82                                             | 1.82                                        |
| D-12    | 84.61                       | 53.47  | 71.29  | 70.44  | 0.75                          | 1.01                            | 0.42                                   | 1.15                                   | 1.33                                 | 1.07                                | 1.86                                             | 0.10                                             | 0.10                                        |
| D-13    | 20.35                       | 9.51   | 26.85  | 10.09  | 0.35                          | 2.66                            | 0.68                                   | 1.28                                   | 1.01                                 | 1.00                                | 0.08                                             | 0.06                                             | 0.06                                        |
| D-14    | 18.43                       | 8.64   | 26.15  | 9.02   | 0.33                          | 2.90                            | 0.65                                   | 1.07                                   | 1.00                                 | 1.00                                | 0.06                                             | 0.06                                             | 0.06                                        |

(1) Radio assay by U-Th method.

(2) Radio assay by Equation 1 method.

1.30, the percent  $\text{U}_3\text{O}_8$  in the sample will be equal to  $K_{2U} C_{2U}$ .

To check the equilibrium condition of the thorium in the ore the count rate contribution of the uranium nuclides on channel 1 can be calculated and subtracted from the total count rate of channel 1. The remaining count rate will be due to the thorium in the ore sample and the thorium equilibrium factor

$$\frac{C_{1T}}{C_{3T}}$$

can be calculated. If the value of this ratio is 0.40 or greater the thorium in the sample will be in equilibrium with its daughters.

In the calculation of the percent  $\text{U}_3\text{O}_8$  in a uranium-thorium composite ore two methods can be used. One is by computing the count rate contribution of the uranium series nuclides on channel 2 as outlined above and then using Formula 1. The other method is to multiply the determination for the percent  $\text{ThO}_2$  in the ore by the

uranium-thorium ratio. When the majority of the count on channel 2 is due to the thorium series of nuclides it is best to use the uranium-thorium ratio method. This is because of the inability to determine accurately the uranium count rate contribution on these channels when the uranium count rate contribution is small compared to the thorium contribution. There is a fairly simple method by which to determine which method to use: When the value of the uranium-thorium ratio is less than 0.20 use the uranium-thorium ratio method, and when the value of the uranium-thorium ratio is greater than 0.20 use the Equation 1 method. Both methods are illustrated in Table 7. When the uranium-thorium ratio is near 0.20 either method should yield about the same result.

15 There are some combinations of uranium series and thorium series nuclides which would be difficult to distinguish. One such combination would be the radium group of the thorium decay series with a uranium-rich uranium ore. On chemical considerations, however, such 20 combinations in nature are almost inconceivable. In any case if they do show up the equilibrium factors, while they may indicate the wrong cause of the state of non-equilibrium, will at least indicate that the ore is not in a state of radioactive equilibrium and therefore cannot 25 be accurately assayed by these methods. Chemical analysis should be used in such cases.

The real value of this method is in the fact that the thorium determination is independent of the equilibrium condition of the uranium in the ore sample. As the equilibrium condition of the uranium can be determined, however, the method is valid for uranium assays. Table 7 lists some results obtained in analyses made by using the methods outlined above. When an assay is rejected the factor that led to its rejection is underlined. A negative 35 thorium equilibrium factor indicates only the radium

groups from the uranium and thorium series are present. D-9 and D-11 illustrate this type of ore. As D-9 and D-11 contain only the radium groups of nuclides from both series the radiometric assays for uranium and thorium will have no value.

60 The uranium equilibrium factor,  $C_{2U}/C_{3U}$ , is a little outside the limits set for equilibrium uranium ore in a few cases in Table 7. This is to be expected when the uranium in a composite ore is a small percentage of that 65 of the thorium. In such cases, personal judgement on the part of the analyst is important. In the case of ores D-3, D-8, and D-14 the author would say that the uranium is in equilibrium. The same is true for the thorium equilibrium factor which in the case of D-4 even becomes negative. Because of the small possibility of non-equilibrium thorium ores occurring with equilibrium uranium ores, the author also would say the thorium in ore D-4 is in equilibrium with its daughters. The main reason for these values wandering outside their 70 limits is that it is very difficult to determine with any accuracy.

curacy the count rate contribution of the uranium or thorium nuclides on a specific channel when the largest share of the count rate on that channel is produced by the other decay series. Especially is this true in the case of channel 1 where self-absorption enters the picture in even low grade ores.

Table 8 lists the values for the various ratios and factors used in assaying composite and other uranium and thorium ores. The values of the factors listed in Table 8 is a function of the efficiency of the equipment involved and the operating conditions of the pulse height analyzer. For example, a wider window width will decrease the proportionality factors. For each particular assaying set-up with a different machine these factors will have to be calculated anew. Assuming equal resolution for all spectrometers used in this work, the new factor will be related to the factor listed in Table 8 by some numerical constant. The value of the uranium equilibrium

TABLE 8.—VARIOUS FACTOR VALUES AND LIMITS USED IN ASSAYING RADIOACTIVE ORES

| Name of Factor                   | Symbol          | Value                             |
|----------------------------------|-----------------|-----------------------------------|
| Uranium Equilibrium Factor       | $C_2/C_3$       | 0.00-∞.                           |
| A. For Equilibrium Uranium Ores. | $C_2/C_3$       | 1.10-1.30.                        |
| B. For Uranium-rich Ores         | $C_2/C_3$       | 3.00-10.0.                        |
| C. For Radium-rich Ores          | $C_2/C_3$       | 0.70-0.95.                        |
| D. For Uranium-Deficient Ores    | $C_2/C_3$       | 0.90-1.00.                        |
| E. For Thorium Ores              | $C_2/C_3$       | 0.30-0.35.                        |
| F. For Thorium-Uranium Ores      | $C_2/C_3$       | 0.30-1.10.                        |
| Composite Ore Factor             | $C_3/C_4$       | 0.55-3.30.                        |
| Thorium Equilibrium Factor       | $C_{1U}/C_{2T}$ | 0.40-0.95.                        |
| Channel 1, Uranium Factor        | $K_{1U}$        | 38.3 c./s. per percent $U_3O_8$ . |
| Channel 2, Uranium Factor        | $K_{2U}$        | 23.8 c./s. per percent $U_3O_8$ . |
| Channel 3, Uranium Factor        | $K_{3U}$        | 20.5 c./s. per percent $U_3O_8$ . |
| Channel 1, Thorium Factor        | $K_{1T}$        | 16.2 c./s. per percent $ThO_2$ .  |
| Channel 2, Thorium Factor        | $K_{2T}$        | 7.2 c./s. per percent $ThO_2$ .   |
| Channel 3, Thorium Factor        | $K_{3T}$        | 24.8 c./s. per percent $ThO_2$ .  |

factor, the composite ore factor, and the thorium equilibrium factor listed in Table 8 will be the same for all gamma-ray scintillation spectrometers assuming the efficiency of all machines in detecting gamma radiation on the various channels bears a linear relationship.

The efficiency of a particular machine is a function of the size of the crystal, the crystal-sample geometry, the size of the sample and the shape of the sample container. If these factors are reproduced as outlined in this application all the factors listed in Table 8 should apply directly.

#### ACCURACY OF ASSAY VALUES

It is difficult to determine the absolute accuracy of the methods outlined in this application. The only standard ores available are chemically assayed ores. The chemical assays used in this application are in most cases routine assays and are not necessarily exact. Some standard ores are available for purchase through the Atomic Energy Commission. The chemical assay of these ores is based on a large number of independent assays from four different laboratories, yet the assay values given for these ores are stated to be accurate to within only 2 percent of the given value.

The first fourteen of the chemical assays listed in Table 4 are the result of very careful chemical analysis, being either Atomic Energy Commission standard ores or ore pulps which were assayed by several independent agencies. The radiometric assay and the chemical assay agree very closely in the case of these ores. The last six ores of Table 4 were chemically analyzed on a routine basis. There is a decided increase in the variance of the radiometric assay and the chemical assay. Considering the small variance of the radio assay and the carefully chemically analyzed samples, there is some justification for assuming that it is the routine chemical assays that are at fault in the case of these last six ores.

Inasmuch as most uranium assaying is done by the fluorimetric method, mention might be made of the accuracy attainable by this method. The following is

quoted from a United States Geological Survey Circular, No. 199, "With careful work uranium may be determined by the fluorescence method with no greater error than 4 percent of the uranium content. Under routine conditions, where speed may be important, the error generally is greater and may amount to plus or minus 8 to 15 percent of the uranium content. When errors occur the results are generally low." This seems to indicate that under routine laboratory conditions an accuracy of plus or minus 10 percent of the actual uranium contained in the sample is good. The accuracy of the assaying methods suggested in this application certainly seems to fall within this range.

A nuclear disintegration is a random phenomenon which is subject to the established methods of statistical analysis. A mathematical analysis of the statistical fluctuations involved in scintillation counting, however, is difficult at best. This is especially true when pulse height analysis is involved, as the statistical fluctuations can arise from several sources in the conversion of gamma radiation into photons of light in the scintillator, in electron emission at the photocathode, in electron multiplication at each dynode, in pulse amplification, and in pulse height discrimination in the analyzer.

To reduce the possibility of error in the assay results due to an incorrect determination of the true disintegration rate of an ore, as long count periods as possible should be used. Too long count periods, however, defeat one of the main reasons for using radioactive assays, that of speed in obtaining analysis results. By gathering a total of about 7500 counts on each channel the probable statistical error in obtaining the true count rate of the ore is in the order of one percent.

When the grade of the ore being assayed was about 0.4 percent  $U_3O_8$  or greater, 7500 counts were gathered on each channel. When the grade of the ore fell below this value a smaller number of counts was gathered so the total assaying time for any one sample did not exceed ten minutes. The accuracy of the result is liable to be reduced in doing this, however, with ores of a grade of 0.10 percent  $U_3O_8$  or less an accuracy of ten or twenty percent of the contained uranium is sufficient for routine assays.

Table 9 contains a list of the results of a succession of independent assays on a single sample of an ore indicating the reproducibility of results with this method. The larger the count gathered, the more accurate the radiometric assay. The ore used in gathering the data for Table 9 was a carefully chemically assayed Colorado Plateau ore. The chemical assay was 0.603 percent  $U_3O_8$ . The average values of the radiometric assays and the mean deviation for the various length of counting runs is also listed in Table 9.

#### CONCLUSIONS

The methods described in this application for analysis of radioactive ores seem to be sufficiently accurate for routine ore analysis. The speed and simplicity of radiometric methods can thus be used to great advantage.

Another significant feature of these methods is their reliability; when it is impossible to assay an ore accurately this fact is indicated. Chemical assaying could be used on these few samples. A majority of the ores normally encountered in routine assaying, however, can be assayed by these energy-discrimination methods. The saving in time is apparent. Important also is the fact that highly skilled technicians are not required to do the analyzing. The use of chemical reagents is not involved in any part of these procedures.

There is an additional saving in time and labor in sample preparation, as the sample need not be finely ground. Crushing to one-quarter inch is sufficient. Weighing of the sample to a tenth of a gram is all that is required, thus, this part of the process, time-consuming in the chemical method, can be markedly shortened.

TABLE 9.—REPRODUCIBILITY OF RADIOMETRIC ASSAYS

| Run No. | Time per Assay | Count Rates (c./s.) |       | Equilibrium Factor, $C_2/C_3$ | Radio Assay, Percent $U_3O_8$ | Average Value of Assays, Percent $U_3O_8$ | Standard Deviation of Assays, Percent $U_3O_8$ |
|---------|----------------|---------------------|-------|-------------------------------|-------------------------------|-------------------------------------------|------------------------------------------------|
|         |                | $C_2$               | $C_3$ |                               |                               |                                           |                                                |
| M-1     | 9 minutes      | 14.34               | 12.40 | 1.16                          | 0.602                         |                                           |                                                |
| M-2     | do             | 14.33               | 12.34 | 1.16                          | 0.602                         |                                           |                                                |
| M-3     | do             | 14.52               | 12.25 | 1.19                          | 0.610                         | 0.606                                     | 0.0034                                         |
| M-4     | do             | 14.55               | 12.75 | 1.14                          | 0.611                         |                                           |                                                |
| M-5     | do             | 14.43               | 12.38 | 1.17                          | 0.606                         |                                           |                                                |
| N-1     | 3 minutes      | 14.28               | 12.80 | 1.11                          | 0.600                         |                                           |                                                |
| N-2     | do             | 14.74               | 12.12 | 1.22                          | 0.619                         |                                           |                                                |
| N-3     | do             | 14.03               | 12.26 | 1.15                          | 0.590                         | 0.605                                     | 0.0100                                         |
| N-4     | do             | 14.25               | 12.46 | 1.14                          | 0.599                         |                                           |                                                |
| N-5     | do             | 14.67               | 12.13 | 1.21                          | 0.615                         |                                           |                                                |
| O-1     | 1 minute       | 14.23               | 12.54 | 1.13                          | 0.598                         |                                           |                                                |
| O-2     | do             | 14.05               | 13.33 | 1.05                          | 0.590                         |                                           |                                                |
| O-3     | do             | 15.06               | 11.72 | 1.28                          | 0.632                         | 0.602                                     | 0.0210                                         |
| O-4     | do             | 14.85               | 12.22 | 1.21                          | 0.624                         |                                           |                                                |
| O-5     | do             | 13.45               | 12.00 | 1.12                          | 0.565                         |                                           |                                                |
| P-1     | 10 seconds     | 15.38               | 11.43 | 1.34                          | 0.645                         |                                           |                                                |
| P-2     | do             | 13.00               | 11.53 | 1.13                          | 0.645                         |                                           |                                                |
| P-3     | do             | 16.56               | 12.20 | 1.36                          | 0.695                         | 0.608                                     | 0.049                                          |
| P-4     | do             | 14.25               | 13.53 | 1.05                          | 0.598                         |                                           |                                                |
| P-5     | do             | 13.30               | 12.40 | 1.07                          | 0.559                         |                                           |                                                |

The fact that a much larger sample is being used in assaying ores by this method means that a more representative sample of the whole is being assayed. The analysis that results by this method is an assay of the complete sample under the scintillometer tube. In chemical assaying seldom more than a gram of ore is used for the analysis. With this energy-discrimination method a 20 or 50 or 100-gram sample can be used. Thus the sample being analyzed is much more representative of the whole, and thus more reliable results can be obtained.

It seems apparent, then, that these methods should be valuable for routine laboratory assaying. On the other hand the equipment involved is light enough for field use. More important, as these methods can yield a continuous and instantaneous assay they can be adapted for use in mill control.

Another important implication of this method is that of being able to assay ores of elements which although not naturally radioactive can be made artificially radioactive through neutron bombardment. Preliminary experiments indicate that ores of copper and gold can be assayed by activating a sample of such an ore with neutrons and then measuring the gamma radiation emitted when the excited atoms disintegrate.

Theoretical considerations indicate that a large number of other materials, such as silver, cobalt, manganese, and tin can also be assayed by activating such materials by neutron bombardment and measuring the characteristic gamma ray that will be emitted by the activated atom.

I accordingly do not desire to be limited in my protection to the specific ores or specific details illustrated and described except as may be necessitated by the appended claims.

I claim:

1. The method of determining equilibrium in uranium and thorium ores comprising measuring the gamma ray radiation given off by key nuclides normally expected to be present in such ore, and dividing the gamma ray radiation intensity from one key nuclide by that from another

25 key nuclide to obtain a value indicative of equilibrium in such ore.

2. The method of determining equilibrium in a uranium ore comprising measuring the gamma ray radiation given off of the key nuclide thorium 230 and the gamma ray radiation given off by the key nuclide lead 214 and dividing the intensity of radiation from the key nuclide thorium 230 by the intensity of radiation from the key nuclide lead 214 to obtain a value indicative of equilibrium in such ore.

35 3. The method of determining equilibrium in a thorium ore comprising measuring the gamma ray radiation given off by the key nuclide thorium 232 and the gamma ray radiation given off by the key nuclide lead 212, and dividing the intensity of radiation from the key nuclide thorium 232 by the intensity of radiation from the key nuclide lead 212 to obtain a value indicative of equilibrium in such ore.

40 4. The steps in the method of assaying composite ores of uranium and thorium comprising measuring the gamma ray intensity at gamma ray energy of approximately 238 kev. and the gamma ray intensity at gamma ray energy of approximately 351 kev., dividing the 238 kev. gamma ray intensity in the 351 kev. gamma ray intensity to obtain a count rate ratio and determining from said 50 count ratio, the ratio of uranium to thorium in such ore.

#### References Cited in the file of this patent

#### UNITED STATES PATENTS

- 55 2,709,754 Davidon May 31, 1955  
2,735,946 Stratford Feb. 21, 1956

#### OTHER REFERENCES

- DiGiovanni: "Scintillation Unit for Drill-Hole Logging," Nucleonics, vol. 11, No. 4, pages 34 to 39 (1953).  
Faul: "Nuclear Geology," John Wiley and Sons, Inc., New York, 1954, pages 250-255.  
Upson et al.: "Analyzing for Low-Energy Gamma Emitters in a Radionuclide Mixture," Nucleonics, vol. 65 13, No. 4, pages 38-42, April 1955.